

Sept. 2, 1930.

A. F. MacLACHLAN

1,774,756

PROCESS IN THE ART OF MANUFACTURING ASPHALT  
BY OXIDIZING HEAVY PETROLEUM HYDROCARBONS

Filed May 12, 1928



*Fig. 1.*



*Fig. 2.*

*Inventor:*

*Allan F. Mac Lachlan*

## UNITED STATES PATENT OFFICE

ALLAN F. MACLACHLAN, OF CHICAGO, ILLINOIS

## PROCESS IN THE ART OF MANUFACTURING ASPHALT BY OXIDIZING HEAVY PETROLEUM HYDROCARBONS

Application filed May 12, 1928. Serial No. 273,045.

This invention relates to a new and improved process in the art of manufacturing asphalt by oxidizing heavy petroleum hydrocarbons. By heavy petroleum hydrocarbons, I means petroleums or petroleum residuums heavier than 24 degrees Baumé or such hydrocarbons mixed with natural or prepared asphalt.

About the only changes in the art of blowing heavy hydrocarbons since the original discoveries of Byerly (U. S. Patent 524,130), and Culmer (U. S. Patent 635,429) have been the use of heavier residuums, higher temperatures, larger volumes of air, and blending.

15 Present day practice is to blow or draw about 9000 cubic feet of air per hour, per ton of eleven degrees Baumé flux for four to eight hours through hydrocarbon flux at 450 to 500 degrees F. This air and fumes are conducted away from the still through a tank to condense part of the oil and then discharged into the atmosphere. This is equivalent to 60 cubic feet of air per minute per 100 gallons charged.

20 25 The disposal of these fumes has been and still is a serious problem in the art as they contain a quantity of oil and a disagreeable smelling gas. In some cases, they are burned or elsewhere they are run into a high stack and discharged into the atmosphere. Ordinarily more than 1½ tons of air are used to produce 1 ton of asphalt and hundreds of tons of fumes are poured into the atmosphere daily.

30 35 I have discovered that asphalt can be made by passing most of these fumes back through the hydrocarbon, mixing them with a relatively small proportion of air or oxidizing gas, the proportion being varied to suit various conditions. If all the fumes are returned the process is very slow but practical results can be secured by the addition of as little as 5% fresh air.

40 45 The apparatus for my process costs less to install and less to operate than most installations, as no extra equipment is needed to carry away the large volume of fumes now handled. The accompanying drawing shows two forms of equipment that may be used to 50 carry out my process, Fig. 1 for blowing air

and Fig. 2 for drawing air through heated heavy hydrocarbons.

A represents a still, heated by burner K, with an ordinary manhole E, pipe lines F and G which may be insulated or cooled, and tank 55 T to collect some of the lighter hydrocarbons that are carried over by the gases. The perforated pipe P permits the oxidizing gases and fumes to bubble through the hydrocarbon. Air can be introduced by partially 60 opening valve D or valve C.

A small opening may be left at H where pipe G enters the still. If valve D is opened, the excess fumes will pass out at H. If valve C is opened, the fresh air is drawn in at H 65 and the small amount of fumes released can be conducted wherever desired. Tank T can be equipped with baffles if desired and insulated if hotter gases are desired.

The lid on manhole E is left on but not 70 bolted down and in case of a flash, the pressure is relieved at this point. The blower B may be on any desirable or convenient level.

The still A is filled about half full of 11 degree Baumé residuum, heat applied and the 75 blower started when a temperature of 300° F. is reached. The temperature is gradually raised to 475° F. and maintained until the asphalt reaches the desired consistency. With a 10-ton charge and a blower 80 delivering 1500 cubic feet of air a minute, it usually takes from four to eight hours blowing to reach 200 degrees melting point, ring and ball test, depending on the air pipe arrangement and the kind of residuum used. 85 For fresh air in the system, I find it convenient to have valves C and D have about one-tenth the area of pipes F and G respectively and to open one of them about half way.

90 From 1% to 5% of the charge usually collects in tank T as a hydrocarbon about eight degrees lighter than the charge. When the charge is finished, this oil may be pumped back into the still and the blower started again for a short time till the previous finished melting point is reached and it will be found that the greater part of the condensed oil is retained in A. Oxygen in relatively small quantity may be introduced into the system at D and greatly increases the speed 95 100

of manufacture. It is a well-known fact that only a small percentage of oxygen is absorbed in oxidizing heavy hydrocarbons.

My process takes care of practically all the fumes or as much as may be found compatible with the speed of manufacture required. It economizes heat as the air retains considerable heat in circulating. It reduces, in fact almost eliminates the oil that is usually carried away in the fumes. It also increases the yield of asphalt by the reabsorption of some of the hydrocarbons in the circulating gases.

Hydrocarbons from different sources produce different asphalts and it is not practical to name them all. The amount of lighter oils that may condense from the fumes may run as high as 30% on some heavy hydrocarbons. I have made asphalt by my process where the sum of the condenser oil and the asphalt checked 99% of the original charge while with the process ordinarily used there would be a loss of 5% to 10% on the same grade of heavy hydrocarbon.

25 I claim:

A new and improved process of manufacturing asphalt by oxidizing heavy petroleum hydrocarbons by continuously circulating the oxidizing gas and the resulting fumes through the original charge, adding as little as 5% of the volume of air used per 100 gallons original charge and maintaining the volume of gases and fumes circulating through the material approximately 50 cubic feet per minute per 35 100 gallons.

ALLAN F. MACLACHLAN.

40

45

50

55

60

65